

## UNITED STATES PATENT OFFICE

2,412,903

## COMPOUNDED LUBRICATING OIL

Robert J. Miller and John T. Rutherford, Berkeley, Calif., assignors, by mesne assignments, to California Research Corporation, San Francisco, Calif., a corporation of Delaware

No Drawing. Application February 1, 1944,  
Serial No. 520,686

10 Claims. (Cl. 252—33.6)

**1** This invention relates to hydrocarbon lubricating oils containing a new and useful combination of addition agents.

This application is a continuation-in-part of our copending application Serial No. 441,964, filed May 6, 1942, now United States Patent No. 2,363,012, issued November 21, 1944.

Hydrocarbon oils, such as petroleum oils, of lubricating viscosity are subject to deterioration at high temperatures and in the presence of oxygen or oxidizing gases, such as the partial combustion products of internal combustion engines. When a straight mineral lubricating oil is subjected to the high temperatures and to the oxidizing gases under high pressure that prevail in aircraft, Diesel and other heavy duty engines, the lubricant undergoes rapid deterioration. This manifests itself in a fouling of the piston by gummy deposits, in the tightening and sticking of piston rings, in wear of moving parts and corrosion of copper-lead and other similar alloy bearings, and, eventually, in engine failure.

It is an object achieved by this invention to provide a hydrocarbon lubricating oil which will resist deterioration caused by heat and oxidation.

It is a further object achieved by this invention to provide a petroleum lubricating oil compounded with such addition agents that it will give more satisfactory performance as a crankcase lubricant for heavy duty service than the uncompounded oil.

It is a particular object achieved by this invention to provide a simple type of compounding for mineral lubricating oils which will provide a marked improvement of the quality of the oil for heavy duty service yet which is more simple and less expensive than many types of compounding used today.

It is a further particular object achieved by the present invention to provide a type of compounding for mineral oil lubricants that is superior to most of the present day compoundings yet which is relatively inexpensive.

These and further objects achieved by the invention will be apparent from the following description and the appended claims.

We have found that a marked improvement in hydrocarbon oils of lubricating viscosity can be effected by incorporating in the oil a small amount of a metal salt of a phenol and of a metal salt of a thiocarbamic acid.

The compounding thus used has been found to produce exceptionally good improvement of mineral lubricating oils and the preferred metal salts used as the compounding are among the least expensive of lubricant addition agents.

**2** Polyvalent metal salts of alkyl substituted phenol and cresols containing 4 to 20 carbon atoms in one or more alkyl groups, and more especially the polyvalent metal salts of bis-(alkyl phenol) sulfides and disulfides and sulfurized polyvalent metal alkyl phenates containing 4 to 20 carbon atoms in one or more alkyl groups, are preferred in the compounding of the present invention. Metal salts of naphthols may also be used. Metal salts of phenols such as disclosed in Reiff, United States Patent 2,197,833; Gardiner et al., United States Patent 2,211,972; Denison et al., United States Patent 2,228,654; Mikeska et al., United States Patent 2,195,539 and Meinert et al., United States Patent 2,230,542 may be used in the combination of this invention.

The metal salts of thiocarbamic acids, which form the second component of the combination of addition agents of this invention, may be represented by the formula



wherein  $R_1$  and  $R_2$  are hydrogen or oil-solubilizing organic groups, at least one  $R$  being an oil-solubilizing organic group;  $X_1$  and  $X_2$  are oxygen or sulfur, at least one  $X$  being sulfur; and  $M$  is a metal. Preferably this second component of the combination of addition agents is a polyvalent metal dithiocarbamate (i. e.,  $M$  is a polyvalent metal and  $X_1$  and  $X_2$  are both sulfur) in which both  $R_1$  and  $R_2$  are groups of hydrocarbon structure, such as polyvalent metal dibutyl dithiocarbamates, polyvalent metal diphenyl dithiocarbamates and polyvalent metal dithiocarbamates derived from cyclic amines such as piperidine and its homologues; e. g., the polyvalent metal petroleum nitrogen base dithiocarbamates produced as described in detail in copending United States Patent application Serial No. 441,964, filed May 6, 1942, now United States Patent #2,363,012. These polyvalent metal petroleum nitrogen base dithiocarbamates are prepared by extracting pyridine bases from cracked naphtha, reducing the extracted bases to the piperidine bases, reacting the piperidine bases with carbon disulfide in aqueous or alcoholic caustic soda or caustic potash and adding a water-soluble polyvalent metal salt to an aqueous solution of the alkali metal petroleum nitrogen base dithiocarbamate to produce double decomposition and precipitation of the polyvalent metal petroleum nitrogen base dithiocarbamate. The polyvalent metal dithiocarbamate may be purified by crystallization from a suitable solvent, such as a light hydrocarbon

thinner. The aforesaid polyvalent metal petroleum nitrogen base dithiocarbamates are the preferred dithiocarbamates of the invention.

In the specification and in the claims, where a formula of a salt, such as



and



is employed, wherein M represents the metal and the residue represents the acid radical, it is to be understood, where M is a polyvalent metal, that the other valences of the metal besides the single valence shown in the formula will be satisfied by the same or other acid radicals, or by an hydroxyl group or groups as in the basic salts. But where a complete formula is given, such as



wherein the subscript a is designated as the valence of M, all the valences of M are accounted for in the formula.

The following specific examples will serve to illustrate the practice and advantages of the present invention.

*Example 1.*—Various uncompounded and compounded petroleum lubricating oils were subjected to test in a single cylinder Lauson gasoline engine. This engine, having a 2 1/8" bore, 2 1/2" stroke, was operated under severe conditions to develop any tendency of the oil to cause piston discoloration, ring sticking and the like: 1200 revolutions per minute, jacket temperature of 375° F., sump oil temperature of 300° F. The engine was inspected after 30 hours and again after 60 hours of operation. The engine inspection included observation of the condition of the piston rings (whether stuck or not) and of the amount of lacquer and gum deposits on the piston skirt. The lacquer and gum deposits on the piston skirt were determined visually and expressed as "Piston Discoloration No." (PD No.). The PD No. rating was accomplished by a widely used method, as follows: The piston skirt surface is divided into the thrust surface and the anti-thrust surface, which are of equal area. Each area is inspected to determine the percentage which is black, percentage dark brown, percentage brown and percentage light brown. Since the darker areas are more serious and represent thicker deposits of gum and lacquer, they are weighted. The weights assigned the black, dark brown, brown and light brown areas are 4, 3, 2 and 1, respectively. The calculation of PD No. is as follows:

|                                                 | Thrust surface | Anti-thrust surface |
|-------------------------------------------------|----------------|---------------------|
| Percentage of area black $\times 4$ .....       | A              | A'                  |
| Percentage of area dark brown $\times 3$ .....  | B              | B'                  |
| Percentage of area brown $\times 2$ .....       | C              | C'                  |
| Percentage of area light brown $\times 1$ ..... | D              | D'                  |
| Total.....                                      | E              | E'                  |

$$\text{PD No.} = E+E'$$

Thus a completely black piston skirt gives a PD

No. of 800 and a completely clean piston skirt gives a PD No. of zero.

Table I

| 5  | Base oil                | Compounding                                                                   | Piston discoloration number |         |
|----|-------------------------|-------------------------------------------------------------------------------|-----------------------------|---------|
|    |                         |                                                                               | 30 hrs.                     | 60 hrs. |
| 10 | S. A. E. 30 blended oil | Nil.....                                                                      |                             | 700     |
|    | Do.....                 | Commercial compounding A                                                      | 80                          | 270     |
|    | Do.....                 | 1% sulfurized Ca cetyl phenate+1% Zn petroleum nitrogen base dithiocarbamate. | 50                          | 150     |
| 15 | Do.....                 | 2.2% "Paranox 56"+1% Zn petroleum nitrogen base dithiocarbamate.              | 55                          | 70      |
|    | Do.....                 | 1% sulfurized Ca cetyl phenate+1% Zn dibutyl dithiocarbamate.                 | 35                          | 55      |
|    | Do.....                 | 1% sulfurized Ca cetyl phenate+1% Cd petroleum nitrogen base dithiocarbamate. | 135                         | 300     |

The S. A. E. 30 blended oil was a blend consisting of 70% solvent treated California naphthenic oil (viscosity index=25) and 30% California paraffinic oil (V. I.=85). Viscosity index of the blend was 57.

In the above table, the 60 hour piston discoloration No. of the base oil was obtained by extrapolation; actually, under the severe conditions of operation, the engine could not be run safely for 60 hours with the uncompounded oil since ring sticking and engine failure would have occurred.

With all of the compounded oils, no ring sticking occurred in 60 hours operation. Commercial compounding A consisted of a phenate, a phosphate and a sulfide and is a compounding which is in wide commercial use in heavy duty oils. The various other compounding agents were as follows:

*Sulfurized Ca cetyl phenate.*—To a mixture of about 237 grams of phenol and 500 grams of a butene polymer (average molecular weight about 194 and boiling range about 375° to 500° F.) are slowly added 140 cc. of 94% sulfuric acid with stirring of the mixture and cooling to maintain the temperature below 65° F. The mixture is agitated for two hours after addition of the acid, cooled to room temperature, diluted with an equal volume of water and heated in an autoclave at 350° F. one hour with agitation. Water is separated and the nonaqueous phase washed with 5% sodium carbonate solution to free it from sulfuric acid, sulfonic acids and unreacted phenol. The product recovered was a high molecular weight, water-insoluble alkyl phenol having an acetyl number of 181.

685 grams of alkylated phenol prepared as described above are agitated six hours at 500°-540° F. with 90 grams of calcium carbide, yielding the calcium alkyl phenate. This is sulfurized by being dissolved in hydrocarbon lubricating oil to form a 50% solution, adding 3/4 gram atom of sulfur per gram mol of calcium alkyl phenate and heating the mixture at 300° to 320° F. for one hour. The reaction mixture is then blown with air until it no longer darkens a copper strip immersed in the hot mixture. The oil solution is then added to the oil which it is desired to compound.

The zinc and cadmium petroleum nitrogen base dithiocarbamates were prepared as described in Example 1 of the aforesaid copending application Serial No. 441,964. They are each

a mixture of compounds which may be represented by the formula



in which the six membered rings containing nitrogen are piperidine rings, each containing one or more alkyl groups (indicated by R and R'), and in which M represents zinc or cadmium.

"Paranox 56" is the trade name of a lubricant addition agent sold by Paraflo Sales Division of Stanco Distributors, Inc. It is the barium salt of a bis-(alkyl phenol)-disulfide.



Zinc dibutyl dithiocarbamate is a compound of the formula



and is commercially available under the trade name of "Dibutyl Zimate."

It is apparent from Table I that the compounding of the present invention not only greatly improves the base oil but that the compounded oil is in the class of very high grade, heavy duty oils. Thus all the oils compounded according to this invention except the last oil (compounded with 1% sulfurized phenate + 1% Cd petroleum nitrogen base dithiocarbamate) were much superior to the oil containing commercial compounding A and even the last oil was nearly as good as the oil containing commercial compounding A.

The advantages flowing from the combination of addition agents of this invention are further shown by the data in the following tables.

In Table II, figures in parentheses were obtained by interpolation and extrapolation. The "Zn Salt" is the same salt as the "Zn petroleum nitrogen base dithiocarbamate" of Table I. The "calcium cetyl phenate" is the unsulfurized calcium phenate described above in connection with the manufacture of sulfurized calcium cetyl phenate; i. e., it is the unsulfurized calcium salt of the alkylated phenol described above.

The oxygen absorption test from which the figures of Table II are taken was carried out as follows: Samples of 50 grams each of base oil and compounded oil were taken and oxygen was bubbled through each sample, the temperature of the oil being maintained at 340° F. and all other conditions, such as oxygen pressure and rate and duration of bubbling, being maintained the same for each sample. Part of the oxygen was absorbed by the oil, the amount absorbed being determined by calculating the difference between unabsoed oxygen and the oxygen fed to the sample of oil.

The Ca cetyl phenate and Zn dithiocarbamate of Table III were the same as the Ca cetyl phenate and Zn salt, respectively, of Table II.

The corrosion test from which the figures of Table III were taken is the test described in United States Patent No. 2,228,658 to Farrington et al. at page 3, right-hand column, lines 27 to 65. Briefly, the test comprises bubbling air through an oil maintained at 300° F. and at 24 hour intervals weighing strips of copper-lead and cadmium-silver bearing-type alloys which are kept immersed in the oil, to determine the loss in weight of the strips. This loss in weight is a measure of the amount of corrosion, being greater the greater the corrosion.

The addition agents of this invention may be used in a wide variety of oils, such as paraffinic, naphthenic and mixed base lubricating oils, oils produced by polymerization of olefin, synthetic lubricating oils, etc. Oils of widely varying viscosity, e. g. 50 S. S. U. at 100° F. to 300 S. S. U.

Table II

| Oil                                              | Cubic centimeters of oxygen absorbed after— |           |          |            |           |           |            |           |
|--------------------------------------------------|---------------------------------------------|-----------|----------|------------|-----------|-----------|------------|-----------|
|                                                  | 0.5 hour                                    | 0.92 hour | 1.0 hour | 1.42 hours | 1.5 hours | 2.0 hours | 2.42 hours | 2.5 hours |
| S. A. E. 30 Pennsylvania (paraffinic) oil.....   | 68                                          |           | 130      |            | 178       | 254       |            | 302       |
| Same+0.5% of Zn salt.....                        | (25)                                        | 38        | (39)     | 45         | (49)      | 57        | 69         | (70)      |
| Same+0.5% of Zn salt+0.5% Ca cetyl phenate.....  | (55)                                        | 66        | (68)     |            | (75)      | (82)      | 90         | (91)      |
| Same+0.25% of Zn salt+0.5% Ca cetyl phenate..... | (60)                                        | 80        | (82)     | 94         | (96)      | 112       | 224        | (350)     |
| Same+0.1% of Zn salt+0.5% Ca cetyl phenate.....  | (60)                                        | 82        | (85)     |            | (99)      | (113)     | 170        | (200)     |

Table III

| Base oil                              | Additives                                           | Weight loss of strip in milligrams |          |          |             |          |          |
|---------------------------------------|-----------------------------------------------------|------------------------------------|----------|----------|-------------|----------|----------|
|                                       |                                                     | Cu-Pb alloy                        |          |          | Cd-Ag alloy |          |          |
|                                       |                                                     | 24 hours                           | 48 hours | 72 hours | 24 hours    | 48 hours | 72 hours |
| California paraffinic base oil.....   | 0.5% Ca cetyl phenate.....                          | 4.5                                | 19.5     | 27.4     | 0           | 0        | 0        |
| Do.....                               | 0.5% Ca cetyl phenate+0.25% Zn dithiocarbamate..... | 1.2                                | 5.3      | 24.4     | 0           | 0        | 0        |
| Do.....                               | 0.5% Ca cetyl phenate+0.5% Zn dithiocarbamate.....  | 0.8                                | 1.0      | 1.9      | 0.1         | 0.1      | 0.3      |
| Pennsylvania paraffinic base oil..... | None.....                                           | 1.6                                | 4.5      | 11.2     | 0.1         | 0.1      | 0.1      |
| Do.....                               | 0.5% Zn dithiocarbamate.....                        | 0.9                                | 1.3      | 1.9      | 0.1         | 0.2      | 0.4      |
| Do.....                               | 0.75% Ca cetyl phenate.....                         | 18.5                               | 107.3    | 166.6    | 5.9         | 111.9    | 215.4    |
| Do.....                               | 0.5% Ca cetyl phenate+0.25% Zn dithiocarbamate..... | 1.0                                | 17.2     | 51.9     | 0.1         | 8.5      | 31.9     |
| Do.....                               | 0.5% Ca cetyl phenate+0.5% Zn dithiocarbamate.....  | 0.7                                | 2.6      | 16.2     | 0.1         | 0.2      | 0.3      |
| Gulf Coast mixed base oil.....        | None.....                                           | 0.2                                | 0.0      | +0.6     | +0.2        | +0.2     | +0.6     |
| Do.....                               | 1% Zn dithiocarbamate.....                          | 0.0                                | 0.0      | +2.2     | +0.1        | +0.1     | 0.0      |
| Do.....                               | 0.5% Ca cetyl phenate.....                          | 17.0                               | 44.0     | 81.5     | 3.7         | 36.4     | 51.7     |
| Do.....                               | 0.5% Ca cetyl phenate+0.5% Zn dithiocarbamate.....  | 0.7                                | 7.6      | 34.7     | 0.1         | 0.4      | 0.1      |

at 210° F. may be compounded with the addition agents of the invention. Amounts of addition agents used will vary with the base oil and the type of service. In general, amounts ranging from about 0.1 to 5 per cent each of phenate and thiocarbamate will be used, preferably about 0.25 to 2 per cent each. (All percentages throughout the specification and claims are percentages by weight based on finished oil unless otherwise indicated.) Concentrates of the addition agents in hydrocarbon lubricating oil, such as petroleum lubricating oil, may be prepared for later blending with more oil to produce the finished oil. For example, concentrates containing up to 25% phenate, up to 25% thiocarbamate and 50% or more hydrocarbon lubricating oil; concentrates containing up to 50% phenate, up to 25% thiocarbamate and 25% or more of hydrocarbon lubricating oil; and concentrates containing up to 25% phenate, up to 50% thiocarbamate and 25% or more hydrocarbon oil, all percentages being by weight based on concentrate, may be prepared.

As stated, polyvalent metal phenates and polyvalent metal thiocarbamates are preferred. Sodium, potassium and lithium phenates and/or thiocarbamates may be used, however; for example, where likelihood of contact with water is very small. Preferred polyvalent metals are the alkaline earth metals (magnesium, calcium, strontium and barium), zinc, cadmium, aluminum and tin. Alkaline earth metal phenates, especially calcium and barium, are preferred and zinc thiocarbamates are preferred.

Thiophenates, such as calcium cetyl thiophenate, may be used in place of or in addition to phenates in the combination of the present invention. Monothiocarbamates may be used in place of or in addition to dithiocarbamates in the combination of the present invention, although dithiocarbamates are preferred. Monothiocarbamates may be of two types: (1) thiocarbamates



and (2) thionocarbamates



Thiocarbamates may be looked upon as derivatives of primary and secondary amines:



wherein both of the R's are hydrocarbon or substituted hydrocarbon groups or one R is a hydrocarbon or substituted hydrocarbon group and the other R is hydrogen. In the first case the thiocarbamate may be looked upon as a derivative of a secondary amine and in the second case, as a derivative of a primary amine. Both types of thiocarbamates may be used in the combination of addition agents of this invention, but the first type (derivatives of secondary amines) is preferred.

The more oil-soluble thiocarbamates are preferred. The good oil solubility of the petroleum base dithiocarbamates is one reason for preferring these compounds. The diphenyl thiocarbamates, such as zinc diphenyl dithiocarbamate, are not as oil-soluble as is desirable, but

their oil solubility may be improved by substitution of alkyl groups on the phenyl groups.

Examples of phenates and thiocarbamates that may be used in combination with each other according to the invention are as follows:

**Phenates.**—Calcium p-tert. amyl phenate; barium 2,4-di-tert. butyl phenate; lithium, magnesium, aluminum and basic barium hexadecyl phenates; calcium "paraffin" phenate (i. e., the normal calcium salt of the product of nuclear condensation of chlorinated paraffin wax with phenol in the presence of a Friedel-Crafts catalyst); barium o-cyclo-hexyl phenate; calcium o-phenyl phenate; calcium hexadecyl chlorophenate; normal barium salt of bis-(tert. amyl phenol)-sulfide; normal barium salt of bis-(4,6-di-tert. butyl-m-cresol)-disulfide; sulfurized calcium 4,6-di-tert. butyl-m-cresylate; calcium hexadecyl amino, nitro and thiophenates; and calcium cetyl hydroxy thiophenate.

**Thiocarbamates.**—Calcium, lead, zinc and cadmium dibutyl dithiocarbamates; zinc methyl octyl dithiocarbamate; zinc dicetyl dithiocarbamate; zinc diethyl thiocarbamate; zinc diethyl thionocarbamate; zinc monooctyl dithiocarbamate; zinc butyl amylphenyl dithiocarbamate; calcium di-cyclohexylphenyl dithiocarbamate; calcium, zinc, cadmium and potassium "petroleum nitrogen base" dithiocarbamates (produced as described in Example 1 of said copending application Serial #441,964, now United States Patent #2,363,012; zinc dibenzyl dithiocarbamate; zinc di-cetylphenyl dithiocarbamate; and zinc di-amylophenyl dithiocarbamate).

Examples of finished oils of this invention are as follows:

*Example 2.*—96-99.5% S. A. E. 30 Pennsylvania oil; 0.25-2% Ba 2,4-di-tert. butyl phenate; 0.25-2% Zn petroleum nitrogen base dithiocarbamate.

*Example 3.*—96-99.5% S. A. E. 30 naphthenic oil; 0.25-2% Ca cetyl phenate; 0.25-2% Zn di-butyl dithiocarbamate.

*Example 4.*—96-99.5% S. A. E. 30 mixed base boil; 0.25-2% sulfurized Ca cetyl phenate; 0.25-2% Cd dibutyl dithiocarbamate.

*Example 5.*—96-99.5% S. A. E. 30 blended paraffinic-naphthenic oil; 0.25-2% Ba salt of bis-(di-ethyl phenol)-sulfide; 0.25-2% Ca di-cetylphenyl dithiocarbamate.

Besides the ingredients indicated, the finished oils may contain other ingredients, such as extreme pressure agents, blooming agents, pour point inhibitors, etc.

We claim:

1. A compounded lubricant comprising a major portion of hydrocarbon lubricating oil, from about 0.1 to about 5% by weight based on the compounded lubricant of an oil-soluble alkaline earth metal phenate and from about 0.1 to 5% by weight based on the compounded lubricant of an oil-soluble zinc thiocarbamate.

2. A compounded lubricant as defined in claim 1 wherein the alkaline earth phenate is a sulfurized salt of an alkyl phenol.

3. A compounded lubricant as defined in claim 1 wherein the alkaline earth phenate is a sulfurized calcium salt of an alkyl phenol.

4. A compounded lubricant as defined in claim 1 wherein the alkaline earth phenate is an alkaline earth metal salt of a bis-(alkyl phenol)-sulfide.

5. A compounded lubricant as defined in claim 1 wherein the alkaline earth phenate is a barium salt of a bis-(alkyl phenol)-sulfide.

6. A compounded lubricant as defined in claim

1 wherein the zinc carbamate is a zinc dithiocarbamate of an aliphatic secondary amine.

7. A compounded lubricant as defined in claim 1 wherein the zinc carbamate is a zinc dithiocarbamate of a mixture of reduced cyclic petroleum nitrogen bases.

8. A compounded lubricant as defined in claim 1 wherein the zinc carbamate is zinc dibutyl di thiocarbamate.

9. A petroleum lubricating oil comprising a 10 major proportion of petroleum lubricating oil, about 0.25 to 2 per cent by weight based on finished oil of a calcium salt of a phenol alkylated with a butene polymer averaging about 16 carbon atoms per molecule and boiling between about 15 375° and 500° F., and about 0.25 to 2 per cent by weight based on finished oil of mixed zinc di-

thiocarbamates of reduced cyclic petroleum nitrogen bases.

10. A lubricant additive capable of inhibiting deterioration of lubricating oils which comprises a concentrated hydrocarbon lubricating oil solution containing from about 5 to about 25% by weight based on the solution of an oil-soluble alkaline earth metal phenate and from about 5 to about 25% by weight based on the solution of an oil-soluble zinc dithiocarbamate, said solution being capable of dilution with hydrocarbon lubricating oil to form a homogeneous mixture containing from 0.1 to 5% by weight of said phenate and from 0.1 to 5% by weight of said carbamate.

ROBERT J. MILLER.  
JOHN T. RUTHERFORD.

**Certificate of Correction**

Patent No. 2,412,903.

ROBERT J. MILLER ET AL.

December 17, 1946.

It is hereby certified that errors appear in the printed specification of the above numbered patent requiring correction as follows: Column 3, line 27, for that portion of the formula reading " $CX_1C_2$ " read  $CX_1X_2$ ; columns 5 and 6, Table III, line 7 under the heading "Additives" for "0.5" read 0.5%; column 8, line 14, for "hexalecyl" read hexadecyl; line 25, for "dithioarbamate" read dithiocarbamate; column 9, lines 8-9, claim 8, for "dithiacarbamate" read dithiocarbamate; and that the said Letters Patent should be read with these corrections therein that the same may conform to the record of the case in the Patent Office.

Signed and sealed this 18th day of February, A. D. 1947.



[SEAL]

**LESLIE FRAZER**

*First Assistant Commissioner of Patents.*